# EUROPEAN PATENT SPECIFICATION

(11) **EP 3 986 574 B1**
(45) Date of publication and mention of the grant of the patent: **23.07.2025**
(21) Application number: 19933338.6
(22) Date of filing: 19.09.2019
(51) Int. Cl.: A62D 1/02, A62D 1/06, A62C 19/00

(54) **IMPROVED FIRE-EXTINGUISHING MIXTURE**
VERBESSERTE FEUERLÖSCHMISCHUNG
MÉLANGE D'EXTINCTION D'INCENDIE AMÉLIORÉ

(30) Priority: 21.06.2019 VN 201900236 U
(43) Date of publication of application: 27.04.2022
(73) Proprietor: Just Throw It, SASU, 94140 Alfortville (FR)
(72) Inventor: NGUYEN, Huan, Ho Chi Minh City (VN)
(74) Representative: Alatis
(86) International application number: PCT/IB2019/057902
(87) International publication number: WO 2020/254869

(56) References cited:
- WO-A1-2013/145207
- WO-A1-2015/020388
- CN-A- 103 007 479
- CN-A- 103 706 062
- CN-A- 104 258 529
- CN-A- 104 474 659
- CN-A- 106 267 635

## Description

### TECHNICAL FIELD

The utility solution relates to an improved fire-extinguishing mixture for throwable fire extinguishers, as well as to a fire extinguisher containing thereof. The fire-extinguishing mixture can extinguish fires of various classes by throwing directly the fire extinguisher containing fire-extinguishing mixture into the fire.

### BACKGROUND

Recently, there is a variety of products referred to as fire extinguishers. Generally, CO2 powder fire extinguishers are difficult to use and heavy. Therefore, it is not convenient to use them in case of a fire. On the other hand, conventional aerosol fire extinguishers can be easily used by anyone, but it is very difficult to use them for dealing with the expanded fire situation. Moreover, throwable fire extinguishers are those that are too easy to use, which contain inorganic foaming fire-extinguishing mixtures with a good extinguishing ability for high temperature fires (175°C and higher). The shell of a fire extinguisher is easy to shatter and distribute the fire-extinguishing mixture, which facilitates the extinguishment of expanded fires. The composition of a fire extinguisher used in the fire extinguisher comprises various agents.

Currently, there have been some types of throwable fire extinguishers available on the market, which have been developed and sold for many years. In particular, these comprise: BONEX fire extinguishers, the throwable fire extinguishers from JAPAN FIRE PROTECT CO.LTD, the fire extinguishers from QINGDAO HUOSHEN EQUIPMENT.CO, the fire extinguishers from FRUNE ZONE CO.LTD, and some other throwable fire extinguishers: FIRE FIGHTER THROWING, TG FIREFIGHTER etc.

An advantage of the prior-art throwable fire extinguishers is their environmental and user friendliness. In particular, the pH of the fire extinguishing solution is about 8, that is, slightly alkaline, thus not causing harm to one's health if swallowed.

CN106267635 A discloses throwable aqueous fire extinguishing compositions in a 650 ml bottle and comprising citric acid, potassium carbonate, sodium bicarbonate, urea, ammonium sulfate, lauryl dimethyl betaine and AFFF/AR (Aqueous Film Forming Foam)/ (Alcohol Resistant) foam extinguishing agent.

However, the prior-art throwable fire extinguishers have the following drawbacks:
- The prior-art throwable fire extinguishers have a not-so-large volume, about 500-650 mL, which have limitation for extinguishment of larger fires.
- The prior-art throwable fire extinguishers on the market contain a fire extinguishing solution that usually has a plurality of ammonium radicals. These ammonium radicals will cause urine odor (smell of urine) for accidental leakage, and breakage into environment during the transport and storage. Such smell is very unpleasant to the users, which makes the deodorization highly time-consuming.
- The prior-art throwable fire extinguishers may be able to extinguish Class A, Class B, and Class C fires only.

### SUMMARY

Given the foregoing, an objective of the utility solution is to develop a safe improved fire-extinguishing mixture that does not have affect to human body and that is an effective fire-extinguishing mixture with extinguishing ability for maximizing the effects of the fire-extinguishing agents, increasing the extinguishing ability, improving user experience during the transport and storage of throwable fire extinguishers.

Accordingly, the utility solution provides an improved fire-extinguishing mixture for throwable fire extinguishers as well as a fire extinguisher containing the same. The fire-extinguishing mixture is able to extinguish Class A, Class B, and Class C (or class F) fires, by throwing directly the fire extinguisher containing fire-extinguishing mixture into to the fire.

According to one aspect of the utility solution, it is provided a fire-extinguishing mixture consisting of:
a. 40% to 55% by weight of potassium carbonate (K₂CO₃),
b. 5 to 10% by weight of sodium bicarbonate (NaHCO₃),
c. 10 to 15% by weight of ammonium bicarbonate (NH₄HCO₃),
d. 5 to 10% by weight of citric acid (C₆H₈O₇),
e. 2 to 7% by weight of sodium lauryl sulfate (C₁₂H₂₅O₄S.Na),
f. 2 to 7% by weight of aqueous film forming foam, and
g. the balance is water (H₂O).

According to another aspect of the utility solution, it is provided a fire extinguisher containing the aforementioned fire-extinguishing mixture.

In an embodiment of this aspect, the utility solution provides a fire extinguisher, having a brittle and fragile plastic shell, that contains the aforementioned fire-extinguishing mixture.

In a more particular embodiment, the previous fire extinguisher contains the aforementioned fire-extinguishing mixture of a 710 mL volume.

According to still another aspect of the utility solution, it is provided a method of producing a fire-extinguishing mixture, the method consisting of the steps of:
- maintaining water at 55-68°C, dissolving 350-440 g of potassium carbonate in a moderate amount of water, until the potassium carbonate is fully dissolved;
- further dissolving 65-80 g of sodium bicarbonate, keeping the temperature of the solution within the range from 55 to 68°C, until the sodium bicarbonate is fully dissolved;
- further dissolving 80-90 g of ammonium bicarbonate, keeping the temperature of the solution within the range from 55 to 68°C, until the ammonium bicarbonate is fully dissolved;
- further dissolving 60-75 g of citric acid, keeping the temperature of the solution within the range from 55 to 68 °C, until the citric acid is fully dissolved;
- cooling the solution to approximately 28°C, then dissolving 40-50 g of sodium lauryl sulfate, until the sodium lauryl sulfate is fully dissolved;
- further dissolving 40-50 g of aqueous film forming foam, until the aqueous film forming foam is fully dissolved;
- adding water into the solution to achieve the volume of 710 mL.

### DETAILED DESCRIPTION

Unless otherwise specified, all of the terms used to describe the utility solution, including the scientific and technical terms, are of the same meaning as understood by those skilled in the art. Further, the definitions of the terms shown herein are indented for better understanding of the disclosure of the utility solution.

As used herein, the expression in singular forms, are intended to include the plural forms and the expression in plural forms also include the singular forms, unless the context clearly indicates otherwise.

The terms "include", "includes", "including" used herein have a similar meaning to "comprise", "comprises", "comprising", and mean to cover all or openended and nonexclusive method steps, features, and other components unmentioned. It should be understood that the terms "include", "inclules", "including" used herein also cover the terms "comprise", "comprises", "comprising".

The expression of numeric ranges with endpoints will include all values and fractions within the corresponding ranges, as well as the said endpoints.

The term "approximately" when used for the numeric values indicates that an approximation to certain degree in calculation and measurement thereof (which is precisely, adjacently, approximately or substantially the same numeric value). If for any reason the inaccuracy resulted from the term "approximately" is not understood by common knowledge in the art, the term "approximately" used herein indicates at least variations from conventional methods of measurement or using of these parameters. For example, the term "generally", "approximately" and "substantially" can be used herein as being within the manufacturing errors. Or, for example, the term "approximately" used herein when changing the amount of a component or a reactant of the utility solution, or when used will indicate variation of the shown amount, is presented by a number that can occur during the common operational and measuring processes used, e.g., when producing concentrates or solutions in practice due to neglection in these processes, or differences in the production, the sources or the purity of the agents used in producing the composition or in implementing the methods, and the like. The term "approximately" also includes the varying amounts due to the balancing of different compositions derived from a particular original mixture. Whether there is change caused by the term "approximately", the claims still include the equivalents to these amounts.

As used herein, a reference to "embodiments" or "an embodiment" means that the particular features, structures or properties are described together with the embodiment will be included at least in one embodiment of the utility solution. As such, the presence of the terms "according to the embodiment" or "according to an embodiment" in various parts of the present specification is not necessary to refer to the same embodiment, but it may be. Furthermore, such features, structures or properties can be combined in any appropriate manner in one or more embodiments, as will be appreciated by a person of ordinary skill in the art when reading the present specification. Furthermore, while some embodiments mentioned herein can include some but not all the features included in other embodiments, the combinations of the features of various embodiments are also within the spirit and scope of the utility solution, and result in different embodiments, as will be appreciated by a person of ordinary skill in the art. For example, in the appended claims, any embodiment of the embodiments claimed can be used as a combination.

Different aspects of the utility solution will be defined in detail in the following sections. Each defined aspect can be combined with another or any other aspects, unless clearly specified otherwise. Particularly, any preferred or advantageous feature can be combined with one or more other preferred or advantageous features. The preferred embodiments of the utility solution will be described below with reference to the accompanying drawings.

Class A fires refer to the fires related to combustible materials such as wood, paper, silk, plastic, textile, waste, and the like.

Class B fires refer to the fires related to flammable liquids, gases, or materials, also referred to as Group B flames.

Class C fires refer to the electrical fires and fires related to electronic devices.

Class K fires, also referred to as kitchen fires (previously referred to as Class F fires, renamed "K" by NFPA 10 in 1998, in The United States of America), are the fires related to flammable liquids such as lards, oils, fats occurring during cooking.

The fire extinguishing solution usually includes ammonium radicals for cooling during the extinguishment. The fire extinguishing solution in high temperature will produce ammonia NH₃. Ammonia usually is unpleasant due to its urine odor, which normally occurs if the extinguisher containing the solution is dropped or broken during transport and storage (in vehicle, building, workshop, etc.).

However, with the fire-extinguishing mixture of the utility solution, the ammonium radicals in the ammonium bicarbonate have been reduced to a proper amount as to alleviate the urine odor of the solution (product) upon breakage during transport and storage of the solution in normal environments (non-extinguishment), but it still maintains the extinguishing efficiency.

In addition, the fire-extinguishing mixture of the utility solution produces a large amount of CO₂ for extinguishment. In particular, potassium carbonate, sodium bicarbonate, ammonium bicarbonate, citric acid thermally react with the fire and create a large amount of CO₂. Particularly, the greater the heat of the fire is, the more CO₂ is produced.

The fire-extinguishing mixture of the utility solution has a very large ratio of K₂CO₃, greatly facilitating the extinguishment of Class F fires (named class "K" by NFPA 10 in 1998, in The United States of America), particularly the fires related to the cooking materials (oils and fats) in cookware.

The fire-extinguishing mixture of the utility solution contains an associated combination of sodium lauryl sulfate and aqueous film forming foam for increasing its extinguishing efficiency . In particular, during the extinguishment, sodium lauryl sulfate and the aqueous film forming foam are combined together, thereby creating foams and water films, and thus rapidly quenching the oxygen source and extinguishing the fire.

The fire extinguisher containing the fire-extinguishing mixture is manufactured with a volume of 710 mL, which is much larger than many other products on the market, in order to increase the extinguishing ability of the fire-extinguishing mixture, thus facilitating the extinguishment of larger fires.

The method of producing the fire-extinguishing mixture according to claim 4 consist of the steps of:
- maintaining water at 55-68 °C, dissolving 350-440 g of potassium carbonate in a moderate amount of water, until the potassium carbonate is fully dissolved;
- further dissolving 65-80 g of sodium bicarbonate, keeping the temperature of the solution within the range from 55 to 68 °C, until the sodium bicarbonate is fully dissolved;
- further dissolving 80-90 g of ammonium bicarbonate, keeping the temperature of the solution within the range from 55 to 68 °C, until the ammonium bicarbonate is fully dissolved;
- further dissolving 60-75 g of citric acid, keeping the temperature of the solution within the range from 55 to 68 °C, until the citric acid is fully dissolved;
- cooling the solution to approximately 28 °C, then dissolving 40-50 g of sodium lauryl sulfate, until the sodium lauryl sulfate is fully dissolved;
- further dissolving 40-50 g of aqueous film forming foam, until the aqueous film forming foam is fully dissolved;
- adding water to the solution to achieve volume of 710 mL.

Then, the fire-extinguishing mixture produced by the aforementioned method is poured into the extinguisher and sealed.

### EXAMPLES

Hereinafter, the utility solution will be described with reference to the examples. These examples are included are only illustrative of certain aspects and embodiments of the utility solution and not intended to be limited in any manner to the utility solution as claimed in the appended claims.

### Example 1 - Preparation of the fire-extinguishing mixture

In an embodiment, a fire-extinguishing mixture is produced by a method consisting of the steps of:
- maintaining water at 55°C, dissolving 350 g potassium carbonate in a moderate amount of water, until the potassium carbonate is fully dissolved;
- further dissolving 65 g of sodium bicarbonate, keeping the temperature of the solution at 55°C, until the sodium bicarbonate is fully dissolved;
- further dissolving 80 g of ammonium bicarbonate, keeping the temperature of the solution at 55°C, until the ammonium bicarbonate is fully dissolved;
- further dissolving 60 g of citric acid, keeping the temperature of the solution at 55°C, until the citric acid is fully dissolved;
- cooling the solution to approximately 28°C, then dissolving 40 g of sodium lauryl sulfate, until the sodium lauryl sulfate is fully dissolved;
- further dissolving 40 g of aqueous film forming foam, until the aqueous film forming foam is fully dissolved;
- adding water to the solution to achieve volume of 710 mL.

As a result, the fire-extinguishing mixture is obtained, which contains:
a. approximately 55% by weight of potassium carbonate (K₂CO₃),
b. approximately 10% by weight of sodium bicarbonate (NaHCO₃),
c. approximately 10% by weight of ammonium bicarbonate (NH₄HCO₃),
d. approximately 10% by weight of citric acid (C₆H₈O₇),
e. approximately 7% by weight of sodium lauryl sulfate (C₁₂H₂₅O₄S.Na),
f. approximately 7% by weight of aqueous film forming foam, and
g. the balance is water (H₂O).

The fire-extinguishing mixture of the utility solution helps to alleviate the urine odor of the fire-extinguishing mixture, increase the extinguishing ability and the re-ignition prevention ability of the fire-extinguishing mixture, and specifically make the fire-extinguishing mixture to be able to extinguish the Class K (Class F) fires.

## Claims

1. A fire-extinguishing mixture consisting of:
a. 40 to 55% by weight of potassium carbonate (K₂CO₃),
b. 5 to 10% by weight of sodium bicarbonate (NaHCO₃),
c. 10 to 15% by weight of ammonium bicarbonate (NH₄HCO₃),
d. 5 to 10% by weight of citric acid (C₆H₈O₇),
e. 2 to 7% by weight of sodium lauryl sulfate (C₁₂H₂₅O₄S.Na),
f. 2 to 7% by weight of aqueous film forming foam, and
g. the balance is water (H₂O).

2. A throwable fire extinguisher containing a fire-extinguishing mixture according to claim . 1.

3. The throwable fire extinguisher according to claim 2, wherein the fire-extinguishing mixture has a volume of 710 mL.

4. A method of producing a fire-extinguishing mixture, to be poured into a throwable fire-extinguisher according to claim 3, consisting of the steps of:
- maintaining water at 55 to 68°C, dissolving 350 to 440 g of potassium carbonate in a moderate amount of water, until the potassium carbonate is fully dissolved;
- further dissolving 65 to 80 g of sodium bicarbonate, keeping the temperature of the solution within the range from 55 to 68°C, until the sodium bicarbonate is fully dissolved;
- further dissolving 80 to 90 g of ammonium bicarbonate, keeping the temperature of the solution within the range from 55 to 68°C, until the ammonium bicarbonate is fully dissolved;
- further dissolving 60 to 75 g of citric acid, keeping the temperature of the solution within the range from 55 to 68°C, until the citric acid is fully dissolved;
- cooling the solution to approximately 28°C, then dissolving 40 to 50 g of sodium lauryl sulfate, until the sodium lauryl sulfate is fully dissolved;
- further dissolving 40 to 50 g of aqueous film forming foam, until the aqueous film forming foam is fully dissolved;
- adding water to the solution to achieve volume of 710 mL.

5. The use of the throwable fire extinguisher according to anyone of claims 2 or 3, to extinguish Class A, Class B and Class C or class F fires, by directly throwing it into the fire.

## Patentansprüche

1. Feuerlöschgemisch, bestehend aus:
a. zu 40 bis 55 Gew.-% Kaliumcarbonat (K₂CO₃),
b. zu 5 bis 10 Gew.-% Natriumbicarbonat (NaHCO₃),
c. zu 10 bis 15 Gew.-% Ammoniumbicarbonat (NH₄HCO₃),
d. zu 5 bis 10 Gew.-% Citronensäure (C₆ H₈O₇),
e. zu 2 bis 7 Gew.-% Natriumlaurylsulfat (C₁₂H₂₅O₄S.Na),
f. zu 2 bis 7 Gew.-% wässrigem filmbildendem Schaum, und
g. der Rest ist Wasser (H₂O).

2. Werfbarer Feuerlöscher, der ein Feuerlöschgemisch nach Anspruch 1 enthält.

3. Werfbarer Feuerlöscher nach Anspruch 2, wobei das Feuerlöschgemisch ein Volumen von 710 ml aufweist.

4. Verfahren zum Herstellen eines Feuerlöschgemischs, das in einen werfbaren Feuerlöscher nach Anspruch 3 eingefüllt werden soll, bestehend aus den Schritten:
- Aufrechterhalten von Wasser bei 55 bis 68 °C, Auflösen von 350 bis 440 g Kaliumcarbonat in einer moderaten Menge Wasser, bis das Kaliumcarbonat vollständig aufgelöst ist;
- ferner Auflösen von 65 bis 80 g Natriumbicarbonat, Halten der Temperatur der Lösung innerhalb des Bereichs von 55 bis 68 °C, bis das Natriumbicarbonat vollständig aufgelöst ist;
- ferner Auflösen von 80 bis 90 g Ammoniumbicarbonat, Halten der Temperatur der Lösung innerhalb des Bereichs von 55 bis 68 °C, bis das Ammoniumbicarbonat vollständig aufgelöst ist;
- ferner Auflösen von 60 bis 75 g Citronensäure, Halten der Temperatur der Lösung innerhalb des Bereichs von 55 bis 68 °C, bis die Citronensäure vollständig aufgelöst ist;
- Abkühlen der Lösung auf etwa 28 °C, dann Auflösen von 40 bis 50 g Natriumlaurylsulfat, bis das Natriumlaurylsulfat vollständig aufgelöst ist;
- ferner Auflösen 40 bis 50 g wässrigen filmbildenden Schaums, bis der wässrige filmbildende Schaum vollständig aufgelöst ist;
- Zugeben von Wasser zu der Lösung, um das Volumen von 710 ml zu erreichen.

5. Verwendung des werfbaren Feuerlöschers nach einem der Ansprüche 2 oder 3, um Feuer von Klasse A, Klasse B und Klasse C oder Klasse F durch direktes Werfen dessen in das Feuer zu löschen.

## Revendications

1. Mélange d'extinction d'incendie composé de :
a. 40 à 55 % en poids de carbonate de potassium (K₂CO₃),
b. 5 à 10 % en poids de bicarbonate de sodium (NaHCO₃),
c. 10 à 15 % en poids de bicarbonate d'ammonium (NH₄HCO₃),
d. 5 à 10 % en poids d'acide citrique (C₆H₈O₇),
e. 2 à 7 % en poids de laurylsulfate de sodium (C₁₂H₂₅O₄S.Na),
f. 2 à 7 % en poids de mousse filmogène aqueuse, et
g. le reste est de l'eau (H₂O).

2. Extincteur à lancer contenant un mélange extincteur d'incendie selon la revendication 1.

3. Extincteur à lancer selon la revendication 2, dans lequel le mélange extincteur a un volume de 710 ml.

4. Procédé de production d'un mélange extincteur d'incendie, destiné à être versé dans un extincteur à lancer selon la revendication 3, comprenant les étapes consistant à :
- maintenir l'eau de 55 à 68 °C, dissoudre 350 à 440 g de carbonate de potassium dans une quantité modérée d'eau, jusqu'à ce que le carbonate de potassium soit complètement dissous ;
- poursuivre avec la dissolution de 65 à 80 g de bicarbonate de sodium, maintenir la température de la solution dans la plage allant de 55 à 68 °C, jusqu'à ce que le bicarbonate de sodium soit entièrement dissous ;
- poursuivre avec la dissolution de 80 à 90 g de bicarbonate d'ammonium, maintenir la température de la solution dans la plage allant de 55 à 68 °C, jusqu'à ce que le bicarbonate d'ammonium soit entièrement dissous ;
- poursuivre avec la dissolution de 60 à 75 g d'acide citrique, maintenir la température de la solution dans la plage allant de 55 à 68 °C, jusqu'à ce que l'acide citrique soit entièrement dissous ;
- refroidir la solution à approximativement 28 °C, puis dissoudre 40 à 50 g de laurylsulfate de sodium, jusqu'à ce que le laurylsulfate de sodium soit entièrement dissous ;
- poursuivre avec la dissolution de 40 à 50 g de mousse filmogène aqueuse, jusqu'à ce que la mousse filmogène aqueuse soit entièrement dissoute ;
- ajouter de l'eau à la solution pour obtenir un volume de 710 ml.

5. Utilisation de l'extincteur à lancer selon l'une quelconque des revendications 2 ou 3, afin d'éteindre des incendies de classe A, de classe B et de classe C ou de classe F, en le jetant directement dans le feu.
